



US006404897B1

(12) **United States Patent**  
Devantier et al.

(10) **Patent No.:** US 6,404,897 B1  
(45) **Date of Patent:** \*Jun. 11, 2002

(54) **CERAMIC METAL MATRIX DIAPHRAGM  
FOR LOUDSPEAKERS**

(75) Inventors: **Allan O. Devantier**, Canyon Country;  
**An D. Nguyen**, West Hills, both of CA  
(US)

(73) Assignee: **Harman International Industries,  
Inc.**, Northridge, CA (US)

(\*) Notice: Subject to any disclaimer, the term of this  
patent is extended or adjusted under 35  
U.S.C. 154(b) by 0 days.

This patent is subject to a terminal disclaimer.

(21) Appl. No.: **09/483,291**

(22) Filed: **Jan. 14, 2000**

**Related U.S. Application Data**

(63) Continuation-in-part of application No. 09/226,087, filed on  
Jan. 5, 1999.

(51) **Int. Cl. 7** ..... **H04R 25/00**

(52) **U.S. Cl.** ..... **381/426; 381/427**

(58) **Field of Search** ..... 181/167, 168,  
181/169, 170, 171, 172, 174; 381/398,  
423, 424, 426, 427, FOR 162, FOR 164

(56) **References Cited**

**U.S. PATENT DOCUMENTS**

3,366,748 A 1/1968 Ashworth

|             |           |                  |
|-------------|-----------|------------------|
| 3,710,040 A | 1/1973    | Swinehart        |
| 4,352,961 A | 10/1982   | Kumada et al.    |
| 4,410,768 A | * 10/1983 | Nakamura et al.  |
| 4,431,873 A | * 2/1984  | Dunn et al.      |
| 5,135,582 A | 8/1992    | Mochizuki et al. |

**OTHER PUBLICATIONS**

“Alluminum Electronic Enclosures” and “Ceramic Components”, *Circle Designfax Cards Nos. 134 and 135*, dated Apr. 1993.

“Ti-Aluminide Blades Tested in GE Engine”, *Aviation Week & Space Technology*, p. 37, Nov. 29, 1993.

“1994 Materials Selector Issue”, *Machine Design*, a Penton Publication, Dec. 1993, pp. 10-13.

“Inside Metal-Cone Speakers”, *Audio Video International*, pp. 24, 26, 28, 30, Nov. 1997.

“Monitor Audio Studio 10”, *Hi-Fi Answers*, Mar. 1990.

\* cited by examiner

*Primary Examiner*—Sinh Tran

*Assistant Examiner*—P. Dabney

(74) *Attorney, Agent, or Firm*—Squire, Sanders & Dempsey L.L.P.

(57) **ABSTRACT**

A method of manufacturing speaker diaphragm for a loudspeaker that has a composite material formed of two layers of ceramic material separated by a light metal substrate and wherein the core is formed by stamping a sheet of standard gauge aluminum to form a speaker core and then deep anodizing the core to obtain a ceramic layer of alumina on each surface ( $Al_2O_3$ ) which is at least about 1 mil. thick.

**9 Claims, 7 Drawing Sheets**





FIG. 1



FIG. 2



FIG. 3



FIG. 4

FIG. 5



FIG. 6



FIG. 7



FIG. 8



FIG. 9



FIG. 10





FIG. 11



FIG. 12



FIG. 13



FIG. 14



*FIG. 15*

## CERAMIC METAL MATRIX DIAPHRAGM FOR LOUDSPEAKERS

### CROSS-REFERENCES TO RELATED APPLICATIONS

This is a continuation-in-part application of Ser. No. 09/226,087 filed Jan. 5, 1999, and having the same inventors and the same title and inventors as the present application.

### BACKGROUND OF THE INVENTION

#### 1. Field of the Invention

The present invention relates in general to loudspeakers and in particular to a diaphragm for a loudspeaker that significantly improves the quality of sound and the usable life of the loudspeaker.

#### 2. Description of Related Art Including Information Disclosed Under 37 CFR 1.97 and 1.98

A typical loudspeaker transducer **10**, as shown in FIG. 1, has a cone **12** and/or dome **14**, diaphragm that is driven by a voice coil **16** that is immersed in a strong magnetic field. The voice coil **16** is electrically connected to an amplifier and, when in operation, the voice coil **16** moves back and forth in response to the electromagnetic forces on the coil caused by the current in the coil, generated by the amplifier, and the stationary magnetic field. The cone **12** and voice coil **16** assembly is typically suspended by a "spider" **18** and a "surround" **13**, a flexible connector to frame **20**. This suspension system allows the cone and coil assembly to move as a finite excursion piston over a limited frequency range. Like all mechanical structures, cones and domes have natural modes or "Mode peaks" commonly called "cone break-up". The frequency at which these modes occur is largely determined by the stiffness, density, and dimensions of the diaphragm, and the amplitude of these modes is largely determined by internal damping of the diaphragm material. These mode peaks are a significant source of audible coloration and, as a result, degrade the performance of the loudspeaker system.

Designers have tended to take two paths to solve the cone break-up problem. For small diaphragms such as those found in dome tweeters, aluminum and titanium are commonly used. In these applications, the dome dimensions can be manipulated such that the first natural modes of the dome are above the frequency range of human hearing. FIG. 2 shows the frequency response of a typical 1" titanium dome tweeter (note the large mode peak **22** at 25 kHz). The amplitude of these modes is usually very high because metals have very little internal damping. For diaphragms larger than approximately 1", the dome modes fall into the audible range. These modes are plainly audible as coloration because of the high amplitude of the modes. FIG. 3 shows the frequency response of a typical 3" titanium dome mid-range speaker (note several large peaks **24**, **26**, and **28** at 11 kHz, 16 kHz, and 18 kHz).

For larger diaphragms, softer materials such as polymers or papers are commonly used. These materials have several natural modes in the band in which they operate. However, the internal damping of these materials is high enough so that most of these modes do not cause audible coloration. The remaining modes are either compensated for in other parts of the loudspeaker system design, resulting in increased costs, or are not addressed at all, resulting in lower performance. FIG. 4 shows the frequency response of a typical 5" woofer with a polypropylene cone (note the large mode peaks **30** and **32** at 4 kHz and 5 kHz).

Many metal diaphragms feature a thin anodized layer. Typically, the metal is anodized to provide a specific color to the visible surface, or to protect the metal from sunlight, humidity, or moisture.

5 Ceramic materials such as alumina or magnesia offer significantly higher stiffness numbers and slightly better internal losses than typical metals such as titanium or aluminum. As a result, the natural modes of diaphragms made of these materials are moved higher in frequency and 10 reduced in amplitude and, thus, reduce audible coloration. For instance, FIG. 14 shows the frequency response of a 5" woofer with a ceramic metal matrix cone of the present invention. Note that the mode peaks **34** and **36** occur at approximately 6.5 kHz and 8.5 kHz. Compare FIG. 14 to 15 FIG. 4. The mode peaks **34** and **36** have moved to a significantly higher frequency than mode peaks **30** and **32** in FIG. 4. This frequency extension allows a more simple and economical roll-off circuit, well known in the art, to be constructed to eliminate the unwanted frequencies.

20 Table I shows the important structural parameters for several materials. Unfortunately, pure ceramics are very brittle and are prone to shattering when used as loudspeaker diaphragms. Additionally, making diaphragms of appropriate dimensions can be very expensive. As a result, pure 25 ceramic loudspeaker diaphragms have not become common.

TABLE I

| Material      | PROPERTIES OF DIAPHRAGM MATERIALS |                       |                |                         |
|---------------|-----------------------------------|-----------------------|----------------|-------------------------|
|               | Young's Modulus (Stiffness)       | Density               | Speed of Sound | Internal Loss (damping) |
| Paper         | $4 \times 10^9$ Pa                | 0.4 g/cm <sup>3</sup> | 1000 m/sec     | 0.06                    |
| Polypropylene | $1.5 \times 10^9$ Pa              | 0.9 g/cm <sup>3</sup> | 1300 m/sec     | 0.08                    |
| Titanium      | $110 \times 10^9$ Pa              | 4.5 g/cm <sup>3</sup> | 4900 m/sec     | 0.003                   |
| Aluminum      | $70 \times 10^9$ Pa               | 2.7 g/cm <sup>3</sup> | 5100 m/sec     | 0.003                   |
| Alumina       | $340 \times 10^9$ Pa              | 3.8 g/cm <sup>3</sup> | 9400 m/sec     | 0.004                   |

### SUMMARY OF THE INVENTION

Thus, the present invention relates to a speaker diaphragm material that is formed of a matrix, or layers, of a light metal such as aluminum, sandwiched between two ceramic layers, 45 preferably aluminum oxide ( $Al_2O_3$ ). The material is particularly useful as a loudspeaker diaphragm. The ceramics,  $Al_2O_3$ , are generally stiffer than metals and also offer improved damping. A loudspeaker diaphragm made of aluminum oxide would offer performance superior to any of the known materials today. Unfortunately, ceramics are also 50 very brittle, and a diaphragm made of pure aluminum oxide would "shatter itself to bits" under normal loudspeaker operations.

Thus, the material of the present invention is made of two 55 layers of ceramic separated by a light metal substrate. Of the common metals, aluminum has the lowest density, making it the ideal substrate. However, there is no known reason why other metals, such as copper, titanium, and the like should not have the same advantages as the use of aluminum.

A skin of alumina, or ceramic, is formed by well-known 60 means, such as anodizing and/or being "grown", on each side of the aluminum core or substrate. Anodizing provides a molecular bond instead of a chemical bond between the substrate and the ceramic material. The alumina thus supplies the strength and the aluminum substrate supplies the resistance to shattering. It has high internal frequency losses. The resulting composite material is less dense and less

brittle than traditional ceramics, yet is significantly stiffer, and has better damping than titanium. It also resists moisture and sunlight better than any polymer and is at least as good as other metals for providing such resistance.

Thus, it is an object of the present invention to provide a loudspeaker diaphragm formed of composite material.

It is also an object of the present invention to provide a loudspeaker diaphragm formed of a composite material that is less dense and less brittle than traditional ceramics, yet it is significantly stiffer and has better damping than titanium.

It is a further object to the present invention to provide a loudspeaker diaphragm that resists moisture and sunlight to a greater degree than any polymer or most metal diaphragms.

It is still another object of the present invention to provide a loudspeaker diaphragm material formed of a composite source of two layers of ceramic material separated by a light metal substrate.

It is still another object to the present invention to provide a speaker diaphragm formed of a layer of light metal, or substrate, having an increased oxide layer on each side and wherein the preferred percentage ratio of ceramic layers to the light metal substrate core is 33½%, 33½%, and 33½%.

It is also an object of the present invention to provide a speaker diaphragm formed of a composite material such as two layers of ceramic material having a thickness of at least about 1 mil. and separated by a light metal substrate.

It is also an object of the present invention to provide a material wherein two layers of ceramic material are separated by a light metal substrate, such as aluminum, and wherein the ceramic layers are formed of  $\text{Al}_2\text{O}_3$ .

#### BRIEF DESCRIPTION OF THE DRAWINGS

These and other features of the present invention will be more fully disclosed when taken in conjunction with the following Detailed Description of the Preferred Embodiment(s) in which like numerals represent like elements and in which:

FIG. 1 is a cross-sectional view of a typical loudspeaker transducer;

FIG. 2 illustrates the frequency response of a typical 1" titanium dome tweeter;

FIG. 3 illustrates the frequency response of a typical 3" titanium dome, mid-range speaker;

FIG. 4 illustrates the frequency response of a typical 5" woofer with a polypropylene cone;

FIG. 5 is a partial cross-sectional view of the present invention applied to a 4" mid-range cone;

FIG. 6 illustrates the Finite Element Analysis (FEA) of a typical 4" mid-range cone constructed of aluminum;

FIG. 7 shows the FEA of the same cone constructed according to the present invention;

FIG. 8 shows the FEA of a cone of the present invention having an aluminum substrate that represents 80% of the total cone thickness;

FIG. 9 shows the FEA of a cone of the present invention having an aluminum substrate that represents 20% of the total cone thickness;

FIG. 10 shows the FEA of a cone of the present invention having an aluminum substrate made of solid ceramic;

FIG. 11 shows the FEA of a 1" dome tweeter as shown in FIG. 2 except with a ceramic metal matrix dome of the present invention;

FIG. 12 shows the frequency response of a 4" mid-range speaker with a traditional aluminum cone;

FIG. 13 shows the frequency response of the same 4" mid-range speaker in FIG. 12 with a ceramic metal matrix cone of the present invention;

FIG. 14 shows the frequency response of the 5" woofer of FIG. 4 formed with the ceramic metal matrix cone of the present invention; and

FIG. 15 shows a flow diagram of the method steps of the present invention.

#### DETAILED DESCRIPTION OF THE PREFERRED EMBODIMENT(S)

The invention shown in FIG. 5 can be described as a composite diaphragm 38 composed of a metal core, or substrate 40, with a layer of ceramic material 42 and 44 on either side in appropriate proportions, so as to minimize both cone break-up (extend the frequency range) and brittleness. FIG. 5 shows the invention in partial cross section as applied to a 4" mid-range cone. In this example a cone of 3 mils. thickness is composed of a substrate of aluminum of 1 mil. thickness and two layers of alumina, each 1 mil. thick, one on each side of the core 40.

The diaphragm 38 is coupled to frame 39 through flexible connector 41 and can be composed of any metal substrate and any ceramic skin. Prior art anodized aluminum cones, which are common, fall into this class. These diaphragms of the prior art are typically 3 mils. thick with a 2.6 mils. thick substrate of aluminum and two 0.2 mil. thick layers of alumina, one on each side of the substrate. In this prior art case, the metal substrate represents approximately 87% of the total thickness of the cone. FIG. 6 shows the Finite Element Analysis of a typical 4" mid-range cone 38 constructed solely of aluminum. The first natural mode peak 44 of the cone distorts the flexible connector 41 and occurs at 8 kHz. FIG. 7 shows the FEA of the same cone constructed in accordance with the present invention while using a 1 mil. aluminum substrate and two 1 mil. layers of alumina, one on each side. The first natural mode 46 of this cone moves all the way to 15 kHz from the 8 kHz of the cone of FIG. 6. In other words, the cone "break-up" occurs at 15 kHz with the present invention as compared to cone "break-up" at 8 kHz of the same prior art speaker.

FIGS. 8 and 9 show the FEA of cones of the present invention with aluminum substrates that represent 80% of the total thickness (FIG. 8) and aluminum substrates that represent 20% of the total thickness (FIG. 9), respectively. As can be seen in Table II, such cone with 80% aluminum substrate has a first "break-up" mode 47 at 12.4 kHz while a cone with 20% aluminum substrate has a first "break-up" mode 49 at 15.95 kHz. For reference, the FEA of a solid ceramic cone is also included as FIG. 10 where the first "break-up" mode 51 occurs at 16 kHz. The optimum thickness for the aluminum substrate of the present invention ranges from 20% to 80% of the total thickness of the diaphragm. For transducer applications, typical thickness of the diaphragm of the present invention ranges from 1 mil. to 25 mils. thickness. As stated, Table II shows the FEA results of various percentages of alumina to the total thickness of the cone from 100% aluminum to 100% alumina.

TABLE II

| Material Type                          | Frequency of the cone's first bending mode | Frequency of the cone's first significant break-up mode | Frequency of the cone's second significant break-up mode | Frequency of the cone's third significant break-up mode |
|----------------------------------------|--------------------------------------------|---------------------------------------------------------|----------------------------------------------------------|---------------------------------------------------------|
| 100% Aluminum                          | 6902 Hz                                    | 8410 Hz                                                 | 11009 Hz                                                 | 12778 Hz                                                |
| 10% Alumina/ 80% Aluminum/ 10% Alumina | 7840 Hz                                    | 12400 Hz                                                | 15060 Hz                                                 | 17340 Hz                                                |
| 33% Alumina/ 33% Aluminum/ 33% Alumina | 9930 Hz                                    | 15060 Hz                                                | 17910 Hz                                                 | 19050 Hz                                                |
| 40% Alumina/ 20% Aluminum/ 40% Alumina | 10100 Hz                                   | 15950 Hz                                                | 18500 Hz                                                 | Above 20000 Hz                                          |
| 100% Alumina                           | 11010 Hz                                   | 16010 Hz                                                | 19050 Hz                                                 | Above 20000 Hz                                          |

As stated earlier, FIG. 2 shows a graph of the frequency response of a 1" dome tweeter with a traditional titanium diaphragm. The graph shows that the first resonant peak 22 occurs at 25 kHz.

FIG. 11 shows the frequency response of the same basic tweeter of FIG. 2 except with a ceramic metal matrix dome of the present invention. On this tweeter the first resonant peak 48 has been moved up to 28 kHz.

FIG. 12 shows the frequency response of a 4" mid-range loudspeaker with a traditional aluminum cone. The graph shows the first resonant peak 50 occurs at 8 kHz. FIG. 13 shows the frequency response of the same basic mid-range loudspeaker except with the ceramic metal matrix cone of the present invention. With this mid-range speaker, the first resonant peak 52 has been moved up to 11 kHz as compared to the 8 kHz frequency of the traditional aluminum cone as shown in FIG. 8.

The graph of FIG. 14, representing a speaker formed with the novel inventive composite material, has been compared earlier with the graph of FIG. 2 for the same traditional speaker.

FIG. 15 shows a flow diagram of the method steps of the present invention.

A 4" mid-range speaker will be used as an example of how to make a ceramic metal matrix diaphragm. The basic shape of the diaphragm is shown in FIG. 5 and is formed of 2 mils. thick aluminum using standard metal forming techniques. The diaphragm is then deep anodized in a well-known manner. In the preferred example, 0.5 mil. of alumina penetrates into the aluminum and 0.5 mil. of alumina is "grown" on the surface of the aluminum on each side, again in a well-known manner. The resulting cone is approximately 3 mils. thick with a 1 mil. thick aluminum substrate and 1 mil. layer of alumina on each side.

Although ceramic/metal/ceramic speakers having a typical thickness of about 3 mils. have their best performance when the speaker is made of 1 mil. ceramic, 1 mil. metal and 1 mil. ceramic, it has been found that an important aspect in increasing the speaker performance is that the ceramic layers be about 1 mil. or greater. Consequently, it has been disclosed that speakers with very good perfor-

mance characteristics can be achieved with speakers of all sizes which have at least 1 mil. of anodizing of each surface, even though the thickness of the metal core is significantly greater than 1 mil.

As examples only, excellent results have been obtained by stamping out the shape of a tweeter speaker from standard gauge 5 mils. sheet metal such as aluminum and then deep anodizing at least  $\frac{1}{2}$  mil. of the metal on each surface. The resulting tweeter diaphragm formed of a composite material will then have a 1 mil. ceramic ( $\text{Al}_2\text{O}_3$ ) layer on one surface, a 4 mil. core and a 1 mil. ceramic ( $\text{Al}_2\text{O}_3$ ) layer on the other surface. Similarly excellent results were obtained stamping out a mid range speaker form from standard gauge 8 mil. metal and anodized to obtain a composite speaker having a 1 mil. layer of ceramic, a 7 mil. core and a 1 mil. layer of ceramic. Excellent results were also achieved by deep anodizing 2 mils. of metal on each surface of an 8 mil. aluminum form to obtain a composite diaphragm having a 4 mil. layer of ceramic, a 4 mil. core and another 4 mil. layer of ceramic.

Using the same techniques a woofer speaker form can be stamped from standard gauge 20 mil. metal and anodized to obtain a composite speaker having a 1 mil. layer of ceramic, a 19 mil. core and a 1 mil. layer of ceramic.

It should be noted that in the past the anodizing depth was limited to about  $\frac{1}{10}$  of a mil. However, by using the substantially thicker standard gauge metal and deep anodizing to at least 1 mil., excellent quality speakers can be achieved which are substantially less expensive.

These ceramic metal matrix diaphragms offer several advantages over the existing technology. One advantage is enabling the use of low cost, simple "roll-off" circuits to eliminate or reduce the audibility of the mode peaks.

Advantages compared to polymers papers, and other "soft" diaphragms:

Significantly higher stiffness to weight ratio.

More consistent performance over a wide range of temperature and humidity. For example, polypropylene's performance changes dramatically with temperature, while paper can be significantly affected by humidity.

Superior immunity to UV light and sunlight.

Superior immunity to water and salt water.

Superior immunity to combustibility.

Advantages compared to aluminum and titanium:

Significantly higher stiffness to weight ratio.

Higher internal damping.

Superior immunity to UV light and sunlight.

Superior immunity to water and salt water.

Offers more color options.

Advantages compared to pure ceramics:

Significantly better resistance to shattering (i.e., less brittle).

Tighter control critical dimensions, including the ability to make very thin walls.

The corresponding structures, materials, acts, and equivalents of all means or step plus function elements in the claims below are intended to include any structure, material, or act for performing the function in combination with other claimed elements as specifically claimed.

What is claimed is:

1. A speaker diaphragm for a loudspeaker comprising: a composite material formed of to layers of ceramic material separated by a light metal substrate to form a speaker diaphragm; and the thickness of the ceramic layers and the light metal substrate having a percentage ratio in the range of from

about 10% to 45% for each ceramic layer and a corresponding 80% to 10% for the lightweight metal substrate.

2. A method of forming a speaker diaphragm for a loudspeaker comprising the steps of:

providing a sheet of light metal having a selected thickness;

forming a speaker core from said sheet of light metal; and forming a ceramic material on each side of said core having a thickness of at least about 1 mil. by anodizing about  $\frac{1}{2}$  mil. of metal on each surface.

3. The method of claim 2 wherein said light metal is aluminum.

4. The method of claim 2 wherein said step of forming a speaker core comprises the step of stamping a speaker core from a sheet of light metal.

5. The method of claim 3 wherein said step of forming a speaker core comprises the step of stamping a speaker core from a sheet of light metal.

6. The method of claim 5 wherein said speaker core is for a tweeter type speaker, said sheet of light metal is 5 mils.

thick and said resulting composite speaker after anodizing has a 1 mil. alumina layer on one side and a 4 mil. core and a 1 mil. alumina layer on the other side.

7. The method of claim 5 wherein said speaker core is for a mid-range type speaker, said sheet of light metal is 8 mils. thick and said resulting composite speaker after anodizing has a 1 mil. alumina layer on one side, a 7 mil. core and a 1 mil. alumina layer on the other side.

8. The method of claim 5 wherein said speaker core is for a mid-range type speaker, said sheet of light metal is 8 mils. thick and said resulting composite speaker after anodizing has a 4 mil. alumina layer on one side, a 4 mil. core and a 4 mil. alumina layer on the other side.

9. The method of claim 5 wherein said speaker core is for a woofer type speaker, said sheet of light metal is 20 mils. thick and said resulting composite speaker after anodizing has a 1 mil. alumina layer on one side and a 19 mil. core and a 1 mil. alumina layer on the other side.

\* \* \* \* \*